

# UNITED STATES PATENT OFFICE.

LOUIS E. BARTON, OF NIAGARA FALLS, NEW YORK, ASSIGNOR TO THE TITANIUM ALLOY MANUFACTURING COMPANY, OF NEW YORK, N. Y., A CORPORATION OF MAINE.

## METHOD OF OBTAINING ZIRCONIUM OXID.

1,351,091.

Specification of Letters Patent. Patented Aug. 31, 1920.

No Drawing.

Application filed September 24, 1919. Serial No. 325,961.

To all whom it may concern:

Be it known that I, LOUIS E. BARTON, a citizen of the United States, and a resident of Niagara Falls, in the county of Niagara 5 and State of New York, have invented certain new and useful Improvements in Methods of Obtaining Zirconium Oxid, of which the following is a specification.

My invention relates to the obtaining of 10 zirconium oxid from materials containing it, as for example from such an ore as baddeleyite, or from zircon (zirconium silicate), in which it may be found, naturally, or otherwise, commingled or associated with one or 15 more of such substances, or impurities, undesired for certain uses, as silica, alumina, iron, titanic, or other oxids, etc.

The objects of my invention comprise the provision of methods whereby zirconium 20 oxid can be, as aforesaid, obtained with industrially practicable speed, directness and economy, and of such purity and other desirable properties as to peculiarly adapt it for an opaquing agent in the production of 25 white enamels; also for use in high grade refractories, pigments, alloys, zirconium salts, etc.

My invention is practised as follows, viz: I bring the above referred to material, or 30 ore, containing zirconium oxid into contact, as by mixing it, preferably preliminarily crushed (except zircon), to about one-half inch size, or smaller, with an oxid reducing agent, preferably a carbonaceous agent, such, 35 for example, as coke, the respective proportions being, within limits, variable as may be indicated:—for example, when coke is employed I usually prefer a ratio of about 20 pounds of coke to 100 pounds of such an 40 ore as baddeleyite, or zircon.

I then charge the mixture gradually into an electric arc furnace at temperature such as to decompose the oxid,—the rate of charging depending upon the composition of the 45 ore, its analysis, and the nature of its above referred to impurities, etc. The best rate of charging is readily determined for a particular charge by a little experimentation and analysis of the resulting product.

50 The result, if the charging be thus gradually and properly made, will, for example when zircon has been mixed with coke, be a product consisting largely, if not essentially, of what I believe to be designatable, and is hereafter designated, as a zirconium cya-

nonitrid; my such products containing by analysis, for example:

|           |              |    |
|-----------|--------------|----|
| Zirconium | 82.0 to 84.0 |    |
| Titanium  | 1.5 to 2.5   | 60 |
| Silica    | .5 to 1.5    |    |
| Iron      | .3 to .5     |    |
| Carbon    | 3.0 to 5.0   |    |
| Nitrogen  | 8.0 to 10.0  |    |

The product is particularly well adapted 65 to treatment by the subsequent steps of my method because it differs in some respects, e. g. as regards the ease with which it is possible to crush, or mill it to even as fine as 350 mesh, and also as regards its composition, 70 as above indicated, from to me known previous carbid or nitrid products obtainable by otherwise than as above described proportioning and smelting the charge.

I continue my gradual charging and smelt- 75 ing until the crucible, or hearth, of the furnace is full, after which I allow the charge to cool and solidify and then remove it from the furnace.

I next crush this product, or solidified 80 melt, consisting preponderatingly of zirconium cyanonitrid, by aid of any appropriate apparatus, such as a jaw crusher, or a rolls and ball mill, or equivalent, capable of reducing it to a condition of fine comminution. 85 The degree of fineness varies as may be indicated by the purpose for which my final zirconium oxid product is to be employed, but it is usually preferable to have it so fine as to pass through a 350 mesh screen. 90

My next step, designed in aid of obtaining my final resulting zirconium oxid product in condition sufficiently purified of undesired substances, such, particularly, as iron compounds, is to subject the above described 95 finely ground material, composed largely, or preponderatingly, of zirconium cyanonitrid, to the action of sulfate of an alkali metal, preferably a neutral sodium sulfate, such as salt cake, or an acid sodium sulfate such as 100 niter cake. To this end I make a thorough mixture in the ratio approximately of 0.75% to 0.80% parts by weight of the sodium sulfate to one part of the zirconium cyanoni- trid. This mixture I charge into an iron ves- 105 sel, and heat until reaction between ingredi- ents of the charge has been started, after which the heat of reaction will usually prove sufficient to melt the mixture and complete 110 the operation. The thus occasioned reactions

result in producing, in the charge, oxids of zirconium and of silicon respectively, in reduction of the sodium sulfate to sodium sulfid, and in the sodium sulfid combining with 5 iron present to form ferro-sodium sulfid. The ignited charge I immediately discharge into water contained in a vessel provided, preferably, with an agitator, and in which I lixiviate the material until its soluble salts, 10 including the ferro-sodium sulfid, are dissolved. The undissolved residue, composed principally of zirconium oxid, settles quickly as a sediment so that I am able to decant the most part of the alkaline sulfid solution, and 15 thus withdraw therefrom the said sediment or residue. The residue I then treat with dilute sulfuric, or other, acid of about 5% strength, as in a bath containing such acid, until the remaining iron compounds, if any, 20 are dissolved. The undissolved residue, *i.e.*, the aforesaid zirconium oxid, I then separate, as by filtration or otherwise, dry it, and finally calcine it at a red heat of from about 600° C. to 700° C., thus producing my sub- 25 stantially pure zirconium oxid final product. In cases involving treatment by my method of a material, or ore, exceptionally impregnated with such undesired substances as iron compounds and from which the 30 highest possible grade of zirconium oxid final product is, for special uses, required, I find it advisable, if not preferable, to, preliminarily to mixing it with the sulfate of the alkaline metal, treat my above de- 35 scribed intermediate product, containing the zirconium cyanonitrid, with dilute sulfuric, or equivalent, acid, as in a bath containing such acid, in order to dissolve and remove the bulk of the iron present. I then wash 40 the residue with cold water, and thereafter mix it with the sulfate of the alkali metal, and, from then on, continue my operation as before described.

The intermediate products derived from 45 this last described treatment of my first, above described, intermediate product, containing zirconium cyanonitrid, by a bath containing dilute sulfuric, or equivalent, acid, preliminarily to my aforesaid treat- 50 ment with the sulfate of the alkaline metal, are, in themselves, and without their treat- 55 ment by other chemical reagents, useful for certain purposes. Their protection I am seeking through the medium of an applica- tion for patent other than this.

Having now described my invention, what I claim as new and desire to secure by Letters Patent is the following, *viz.:*

1. In obtaining zirconium oxid, from a

material containing an undesired substance, 60 the steps which consist in melting said material with a carbonaceous reducing agent to production of zirconium cyanonitrid; and subjecting the resulting product to the action of sulfate of an alkali metal. 65

2. In obtaining zirconium oxid from a material containing an undesired substance, the steps which consist in melting said material with a carbonaceous reducing agent to production of zirconium cyanonitrid; 70 treating the resulting product to a bath containing a dilute acid; withdrawing the undissolved residue; and subjecting it to the action of sulfate of an alkali metal.

3. In obtaining zirconium oxid from a 75 material containing an undesired substance, the steps which consist in melting said material with a carbonaceous reducing agent to production of zirconium cyanonitrid; subjecting the resulting product to the action of sulfate of an alkali metal, and there- 80 after dissolving remaining iron compounds in dilute acid.

4. The method of obtaining zirconium 85 oxid, from a material containing an undesired substance, which comprises: melting said material with a carbonaceous reducing agent to production of zirconium cyanoni- 90 trid; subjecting the resulting product to the action of sulfate of an alkali metal; sub- 95 jecting the resulting product to an aqueous bath; withdrawing from said bath its sediment, or undissolved residue; subjecting it to the action of another bath containing a dilute acid; separating from said last men- 100 tioned bath its undissolved residue; and cal- cining it.

5. The method of obtaining zirconium 105 oxid from a material containing an undesired substance, which comprises: melting 100 said material with a carbonaceous reducing agent to production of zirconium cyanoni- 110 trid; treating the resulting product to a bath containing a dilute acid; withdrawing and washing the undissolved residue; sub- 115 jecting said residue to the action of sulfate of an alkali metal; subjecting the resulting product to an aqueous bath; withdrawing from said bath its sediment, or undissolved residue; subjecting this last mentioned residue to the action of a bath containing a dilute acid; separating from said last men- 120 tioned bath its undissolved residue; and cal- cining it.

LOUIS E. BARTON.

Witnesses:

TOM C. GRAHAM,  
CARL P. REISIG.